



US008431318B2

(12) **United States Patent**  
**Vanbesien et al.**

(10) **Patent No.:** **US 8,431,318 B2**  
(b5) **Date of Patent:** **Apr. 30, 2013**

(54) **TONER COMPOSITIONS AND PROCESSES**

(75) Inventors: **Daryl W. Vanbesien**, Burlington (CA); **Allan K. Chen**, Oakville (CA); **Kimberly D. Nosella**, Mississauga (CA); **Cuong Vong**, Hamilton (CA); **Karen Ann Moffat**, Brantford (CA); **Richard P. N. Veregin**, Mississauga (CA); **Valerie M. Farrugia**, Oakville (CA)

(73) Assignee: **Xerox Corporation**, Norwalk, CT (US)

(\*) Notice: Subject to any disclaimer, the term of this patent is extended or adjusted under 35 U.S.C. 154(b) by 427 days.

(21) Appl. No.: **12/757,321**

(22) Filed: **Apr. 9, 2010**

(65) **Prior Publication Data**

US 2011/0250535 A1 Oct. 13, 2011

(51) **Int. Cl.**

**G03G 9/00** (2006.01)

(52) **U.S. Cl.**

USPC ..... **430/137.14**; 430/109.4

(58) **Field of Classification Search** ..... 430/108.1, 430/108.8, 109.1, 109.4, 110.2, 137.1, 137.14  
See application file for complete search history.

(56) **References Cited**

## U.S. PATENT DOCUMENTS

|             |         |                  |
|-------------|---------|------------------|
| 3,590,000 A | 6/1971  | Palermi et al.   |
| 3,681,106 A | 8/1972  | Burns et al.     |
| 3,800,588 A | 4/1974  | Larson et al.    |
| 3,847,604 A | 11/1974 | Hagenbach et al. |
| 4,295,990 A | 10/1981 | Verbeek et al.   |
| 4,298,672 A | 11/1981 | Lu               |
| 4,338,390 A | 7/1982  | Lu               |
| 4,533,614 A | 8/1985  | Fukumoto et al.  |

|             |         |                   |
|-------------|---------|-------------------|
| 4,845,006 A | 7/1989  | Matsubara et al.  |
| 4,863,824 A | 9/1989  | Uchida et al.     |
| 4,863,825 A | 9/1989  | Yoshimoto et al.  |
| 4,917,983 A | 4/1990  | Uchida et al.     |
| 4,931,370 A | 6/1990  | Amaya et al.      |
| 4,933,252 A | 6/1990  | Nishikawa et al.  |
| 4,935,326 A | 6/1990  | Creatura et al.   |
| 4,937,166 A | 6/1990  | Creatura et al.   |
| 4,957,774 A | 9/1990  | Doi et al.        |
| 4,973,539 A | 11/1990 | Sacripante et al. |
| 4,980,448 A | 12/1990 | Tajiri et al.     |
| 4,981,939 A | 1/1991  | Matsumura et al.  |
| 4,988,794 A | 1/1991  | Kubo et al.       |
| 5,057,596 A | 10/1991 | Kubo et al.       |
| 5,143,809 A | 9/1992  | Kaneko et al.     |
| 5,227,460 A | 7/1993  | Mahabadi et al.   |
| 5,236,629 A | 8/1993  | Mahabadi et al.   |
| 5,290,654 A | 3/1994  | Sacripante et al. |
| 5,302,486 A | 4/1994  | Patel et al.      |
| 5,330,874 A | 7/1994  | Mahabadi et al.   |
| 5,376,494 A | 12/1994 | Mahabadi et al.   |
| 5,480,756 A | 1/1996  | Mahabadi et al.   |
| 5,500,324 A | 3/1996  | Mahabadi et al.   |
| 5,527,658 A | 6/1996  | Hopper et al.     |
| 5,601,960 A | 2/1997  | Mahabadi et al.   |

(Continued)

## OTHER PUBLICATIONS

U.S. Appl. No. 12/248,939, filed Oct. 10, 2008, Vanbesien et al.

Primary Examiner — Stewart Fraser

(74) Attorney, Agent, or Firm — MDIP LLC

(57) **ABSTRACT**

The present disclosure provides processes for producing polyester toners by emulsion aggregation where the resulting toner particles have high pigment loadings and desired circularity. The methods include adding a metal, in embodiments a metal compound, at the beginning of coalescence, which speeds the coalescence process and produces toner particles having a desired size and circularity for use in electrophotographic imaging systems.

**20 Claims, 4 Drawing Sheets**

## U.S. PATENT DOCUMENTS

|              |         |                    |                   |         |                           |
|--------------|---------|--------------------|-------------------|---------|---------------------------|
| 5,629,121 A  | 5/1997  | Nakayama           | 7,329,476 B2      | 2/2008  | Sacripante et al.         |
| 5,650,484 A  | 7/1997  | Hawkins et al.     | 7,546,069 B2      | 6/2009  | Kumar et al.              |
| 5,750,909 A  | 5/1998  | Hawkins et al.     | 2006/0216626 A1   | 9/2006  | Sacripante et al.         |
| 6,214,507 B1 | 4/2001  | Sokol et al.       | 2007/0243478 A1 * | 10/2007 | Maeyama .....             |
| 6,326,119 B1 | 12/2001 | Hollenbaugh et al. | 2008/0107990 A1   | 5/2008  | Field et al.              |
| 6,358,657 B1 | 3/2002  | Silence et al.     | 2008/0236446 A1   | 10/2008 | Zhou et al.               |
| 6,359,105 B1 | 3/2002  | Ianni et al.       | 2009/0047593 A1   | 2/2009  | Vanbesien et al.          |
| 6,592,913 B2 | 7/2003  | Cook et al.        | 2009/0274499 A1 * | 11/2009 | Kovacs et al. .....       |
| 6,593,053 B1 | 7/2003  | Chang et al.       | 2010/0055598 A1 * | 3/2010  | 399/335 Zhou et al. ..... |

\* cited by examiner



*FIG. 1A*



*FIG. 1B*



FIG. 2



FIG. 3



FIG. 4

## TONER COMPOSITIONS AND PROCESSES

## BACKGROUND

The present disclosure relates to processes useful in providing toners suitable for electrophotographic apparatuses, including digital, image-on-image, and similar apparatuses.

Toner blends containing crystalline or semi-crystalline polyester resins with an amorphous resin have recently been shown to provide very desirable ultra low melt fusing, which is important for both high-speed printing and lower fuser power consumption. These types of toners containing crystalline polyesters have been demonstrated suitable for both emulsion aggregation (EA) toners, and in conventional jetted toners. Combinations of amorphous and crystalline polyesters may provide toners with relatively low-melting point characteristics (sometimes referred to as low-melt, ultra low melt or ULM), which allows for more energy-efficient and faster printing.

The development of highly pigmented toners may affect the toner formation process, with difficulties arising in forming toner particles having a desired size and shape.

Improved methods for producing toner remain desirable.

## SUMMARY

The present disclosure provides processes for producing toners and toners produced thereby. In embodiments, a process of the present disclosure includes contacting at least one polyester resin with at least one colorant, at least one surfactant, and an optional wax to form an emulsion possessing small particles; aggregating the small particles; adding a metal compound including a metal such as copper, iron, and alloys thereof to the small particles; coalescing the aggregated particles to form toner particles; and recovering the toner particles, wherein the toner particles possess a volume average diameter of from about 3 microns to about 10 microns.

In other embodiments, a process of the present disclosure may include contacting at least one amorphous resin with at least one crystalline resin, at least one colorant, at least one surfactant, and an optional wax to form an emulsion possessing small particles; aggregating the small particles; adding to the small particles a metal compound including nitrates, sulfates, halides, acetates, phosphates, oxides, hydroxides, carbonates, and combinations thereof, possessing a metal such as copper, iron, and alloys thereof; coalescing the aggregated particles to form toner particles; and recovering the toner particles, wherein the toner particles possess a volume average diameter of from about 3 microns to about 10 microns.

In other embodiments, a process of the present disclosure may include contacting at least one amorphous resin with at least one crystalline resin, at least one colorant, at least one surfactant, and an optional wax to form an emulsion possessing small particles; aggregating the small particles; adding to the small particles a metal compound including nitrates, sulfates, halides, acetates, phosphates, oxides, hydroxides, carbonates, and combinations thereof, possessing a metal such as copper, iron, and alloys thereof; coalescing the aggregated particles for a period of time of from about 0.5 hours to about 5 hours to form toner particles; and recovering the toner particles, wherein the colorant includes dyes, pigments, combinations of dyes, combinations of pigments, and combinations of dyes and pigments, present in an amount of from about 4 percent to about 40 percent by weight of the toner, and wherein the toner particles possess a volume average diam-

eter of from about 3 microns to about 10 microns, and a circularity of from about 0.95 to about 0.998.

In embodiments, the toner particles may then be applied to a substrate and fused to the substrate, wherein an image formed with the toner has a toner pile height from about 0.5 microns to about 7 microns.

## BRIEF DESCRIPTION OF THE FIGURES

- 10 Various embodiments of the present disclosure will be described herein below with reference to the figures wherein:  
 FIG. 1 depicts formation of an image with a toner of the present disclosure (FIG. 1B) compared with a conventional toner (FIG. 1A);  
 15 FIG. 2 is a graph depicting circularity obtained for toner particles as a function of time during coalescence for polyester EA toners produced in the various Examples;  
 FIG. 3 is a graph depicting charging results obtained for the toners of the Examples; and  
 20 FIG. 4 is a graph depicting charging results obtained for a commercially available magenta toner.

## DETAILED DESCRIPTION OF EMBODIMENTS

25 The present disclosure provides processes for the preparation of toner particles which may avoid problems arising in the formation of highly pigmented particles. In embodiments, a transition metal compound, which may be a powder and/or a transition metal salt, may be added to toner particles during 30 an emulsion aggregation synthesis to facilitate rapid coalescence of the toner particles, with the toner particles possessing a high degree of circularity.

Toners of the present disclosure may include a latex resin in combination with a pigment. While the latex resin may be 35 prepared by any method within the purview of those skilled in the art, in embodiments the latex resin may be prepared by emulsion polymerization methods, including semi-continuous emulsion polymerization, and the toner may include emulsion aggregation toners. Emulsion aggregation involves 40 aggregation of both submicron latex and pigment particles into toner size particles, where the growth in particle size is, for example, in embodiments from about 0.1 micron to about 15 microns.  
 Resins

45 Any toner resin may be utilized in the processes of the present disclosure. Such resins, in turn, may be made of any suitable monomer or monomers via any suitable polymerization method. In embodiments, the resin may be prepared by a method other than emulsion polymerization. In further embodiments, the resin may be prepared by condensation polymerization.

The toner composition of the present disclosure, in 55 embodiments, includes an amorphous resin. The amorphous resin may be linear or branched. In embodiments, the amorphous resin may include at least one low molecular weight amorphous polyester resin. The low molecular weight amorphous polyester resins, which are available from a number of sources, can possess various melting points of, for example, from about 30° C. to about 120° C., in embodiments from 60 about 75° C. to about 115° C., in embodiments from about 100° C. to about 110° C., and/or in embodiments from about 104° C. to about 108° C. As used herein, the low molecular weight amorphous polyester resin has, for example, a number average molecular weight ( $M_n$ ), as measured by gel permeation chromatography (GPC) of, for example, from about 1,000 to about 10,000, in embodiments from about 2,000 to 65 about 8,000, in embodiments from about 3,000 to about

7,000, and in embodiments from about 4,000 to about 6,000. The weight average molecular weight ( $M_w$ ) of the resin is 50,000 or less, for example, in embodiments from about 2,000 to about 50,000, in embodiments from about 3,000 to about 40,000, in embodiments from about 10,000 to about 30,000, and in embodiments from about 18,000 to about 21,000, as determined by GPC using polystyrene standards. The molecular weight distribution ( $M_w/M_n$ ) of the low molecular weight amorphous resin is, for example, from about 2 to about 6, in embodiments from about 3 to about 4. The low molecular weight amorphous polyester resins may have an acid value of from about 8 to about 20 mg KOH/g, in embodiments from about 9 to about 16 mg KOH/g, and in embodiments from about 10 to about 14 mg KOH/g.

Examples of linear amorphous polyester resins which may be utilized include poly(propoxylated bisphenol A co-fumarate), poly(ethoxylated bisphenol A co-fumarate), poly(butoxylated bisphenol A co-fumarate), poly(co-propoxylated bisphenol A co-ethoxylated bisphenol A co-fumarate), poly(1,2-propylene fumarate), poly(propoxylated bisphenol A co-maleate), poly(ethoxylated bisphenol A co-maleate), poly(butoxylated bisphenol A co-maleate), poly(co-propoxylated bisphenol A co-ethoxylated bisphenol A co-maleate), poly(1,2-propylene maleate), poly(propoxylated bisphenol A co-itaconate), poly(ethoxylated bisphenol A co-itaconate), poly(butoxylated bisphenol A co-itaconate), poly(co-propoxylated bisphenol A co-ethoxylated bisphenol A co-itaconate), poly(1,2-propylene itaconate), and combinations thereof.

In embodiments, a suitable linear amorphous polyester resin may be a poly(propoxylated bisphenol A co-fumarate) resin having the following formula (I):



wherein  $m$  may be from about 5 to about 1000.

An example of a linear propoxylated bisphenol A fumarate resin which may be utilized as a latex resin is available under the trade name SPARIITM from Resana SIA Industrias Quimicas, Sao Paulo Brazil. Other suitable linear resins include those disclosed in U.S. Pat. Nos. 4,533,614, 4,957,774 and 4,533,614, which can be linear polyester resins including terephthalic acid, dodecylsuccinic acid, trimellitic acid, fumaric acid and alkyloxylation bisphenol A, such as, for example, bisphenol-A ethylene oxide adducts and bisphenol-A propylene oxide adducts. Other propoxylated bisphenol A terephthalate resins that may be utilized and are commercially available include GTU-FC115, commercially available from Kao Corporation, Japan, and the like.

In embodiments, the low molecular weight amorphous polyester resin may be a saturated or unsaturated amorphous polyester resin. Illustrative examples of saturated and unsaturated amorphous polyester resins selected for the process and particles of the present disclosure include any of the various amorphous polyesters, such as polyethylene-terephthalate, polypropylene-terephthalate, polybutylene-terephthalate, polypentylene-terephthalate, polyhexalene-terephthalate, polyheptadene-terephthalate, polyoctalene-terephthalate, polyethylene-isophthalate, polybutylene-isophthalate, polypropylene-isophthalate, polyhexalene-isophthalate, polyheptadene-isophthalate, polyoctalene-isophthalate, polyethylene-sebacate, polypropylene sebacate, polybutylene-sebacate, polyethylene-adipate, polypropylene-adipate, polybutylene-adipate, polypropylene-adipate, polyhexalene-adipate, polyheptadene-adipate, polyoctalene-adipate, polyethylene-glutarate, polypropylene-glutarate, polybutylene-glutarate, polypentylene-glutarate, polyhexalene-glutarate, polyheptadene-glutarate, polyoctalene-glutarate, polyethylene-pimelate, polypropylene-pimelate, polybutylene-pimelate, polypentylene-pimelate, polyhexalene-pimelate, polyheptadene-pimelate, poly(ethoxylated bisphenol A-fumarate), poly(ethoxylated bisphenol A-succinate), poly(ethoxylated bisphenol A-adipate), poly(ethoxylated bisphenol A-glutarate), poly(ethoxylated bisphenol A-terephthalate), poly(ethoxylated bisphenol A-isophthalate), poly(ethoxylated bisphenol A-dodecylsuccinate), poly(propoxylated bisphenol A-fumarate), poly(propoxylated bisphenol A-adipate), poly(propoxylated bisphenol A-glutarate), poly(propoxylated bisphenol A-terephthalate), poly(propoxylated bisphenol A-isophthalate), poly(propoxylated bisphenol A-dodecylsuccinate), SPAR (Dixie Chemicals), BECKOSOL (Reichhold Inc), ARAKOTE (Ciba-Geigy Corporation), HETRON (Ashland Chemical), PARAPLEX (Rohm & Haas), POLYLITE (Reichhold Inc), PLASTHALL (Rohm & Haas), CYGAL (American Cyanamide), ARMCO (Armco Composites), ARPOL (Ashland Chemical), CELANEX (Celanese Eng), RYNITE (DuPont), STYPOL (Freeman Chemical Corporation) and combinations thereof. The resins can also be functionalized, such as carboxylated, sulfonated, or the like, and particularly such as sodio sulfonated, if desired.

The low molecular weight linear amorphous polyester resins are generally prepared by the polycondensation of an organic diol, a diacid or diester, and a polycondensation catalyst. The low molecular weight amorphous resin is generally present in the toner composition in various suitable amounts, such as from about 60 to about 90 weight percent, in embodiments from about 50 to about 65 weight percent, of the toner or of the solids.

Examples of organic diols selected for the preparation of low molecular weight resins include aliphatic diols with from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,12-dodecanediol, and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like. The aliphatic diol is, for example, selected in an amount of from about 45 to about 50 mole percent of the resin, and the alkali sulfo-aliphatic diol can be selected in an amount of from about 1 to about 10 mole percent of the resin.

Examples of diacid or diesters selected for the preparation of the low molecular weight amorphous polyester include dicarboxylic acids or diesters such as terephthalic acid, phthalic acid, isophthalic acid, fumaric acid, maleic acid, itaconic acid, succinic acid, succinic anhydride, dodecylsuccinic acid, dodecylsuccinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethyl-

succinate, dimethylfumarate, dimethylmaleate, dimethylglutarate, dimethyladipate, dimethyl dodecylsuccinate, dimethyl dodecylsuccinate, and mixtures thereof. The organic diacid or diester is selected, for example, from about 45 to about 52 mole percent of the resin.

Examples of suitable polycondensation catalyst for either the low molecular weight amorphous polyester resin include tetraalkyl titanates, dialkyltin oxide such as dibutyltin oxide, tetraalkyltin such as dibutyltin dilaurate, dialkyltin oxide hydroxide such as butyltin oxide hydroxide, aluminum alkoxides, alkyl zinc, dialkyl zinc, zinc oxide, stannous oxide, or mixtures thereof; and which catalysts may be utilized in amounts of, for example, from about 0.01 mole percent to about 5 mole percent based on the starting diacid or diester used to generate the polyester resin.

The low molecular weight amorphous polyester resin may be a branched resin. As used herein, the terms "branched" or "branching" includes branched resin and/or cross-linked resins. Branching agents for use in forming these branched resins include, for example, a multivalent polyacid such as 1,2,4-benzene-tricarboxylic acid, 1,2,4-cyclohexanetricarboxylic acid, 2,5,7-naphthalenetetracarboxylic acid, 1,2,5-hexanetricarboxylic acid, 1,3,5-dicarboxyl-2-methyl-2-methylene-carboxylpropane, tetra(methylene-carboxyl)methane, and 1,2,7,8-octanetetracarboxylic acid, acid anhydrides thereof, and lower alkyl esters thereof, 1 to about 6 carbon atoms; a multivalent polyol such as sorbitol, 1,2,3,6-hexanetetrol, 1,4-sorbitane, pentaerythritol, dipentaerythritol, tri-pentaerythritol, sucrose, 1,2,4-butanetriol, 1,2,5-pentatriol, glycerol, 2-methylpropanetriol, 2-methyl-1,2,4-butanetriol, trimethylolethane, trimethylolpropane, 1,3,5-trihydroxymethylbenzene, mixtures thereof, and the like. The branching agent amount selected is, for example, from about 0.1 to about 5 mole percent of the resin.

Linear or branched unsaturated polyesters selected for the *in situ* pre-wise reactions between both saturated and unsaturated diacids (or anhydrides) and dihydric alcohols (glycols or diols). The resulting unsaturated polyesters are reactive (for example, crosslinkable) on two fronts: (i) unsaturation sites (double bonds) along the polyester chain, and (ii) functional groups such as carboxyl, hydroxy, and the like groups amenable to acid-base reactions. Typical unsaturated polyester resins are prepared by melt polycondensation or other polymerization processes using diacids and/or anhydrides and diols.

In embodiments, the low molecular weight amorphous polyester resin or a combination of low molecular weight amorphous resins may have a glass transition temperature of from about 30° C. to about 80° C., in embodiments from about 35° C. to about 70° C. In further embodiments, the combined amorphous resins may have a melt viscosity of from about 10 to about 1,000,000 Pa\*S at about 130° C., in embodiments from about 50 to about 100,000 Pa\*S.

The monomers used in making the selected amorphous polyester resin are not limited, and the monomers utilized may include any one or more of, for example, ethylene, propylene, and the like. Known chain transfer agents, for example dodecanethiol or carbon tetrabromide, can be utilized to control the molecular weight properties of the polyester. Any suitable method for forming the amorphous or crystalline polyester from the monomers may be used without restriction.

The amount of the low molecular weight amorphous polyester resin in a toner particle of the present disclosure, whether in core, any shell, or both, may be present in an

amount of from 25 to about 50 percent by weight, in embodiments from about 30 to about 45 percent by weight, and in embodiments from about 35 to about 43 percent by weight, of the toner particles (that is, toner particles exclusive of external additives and water).

In embodiments, the toner composition includes at least one crystalline resin. As used herein, "crystalline" refers to a polyester with a three dimensional order. "Semicrystalline resins" as used herein refers to resins with a crystalline percentage of, for example, from about 10 to about 90%, in embodiments from about 12 to about 70%. Further, as used hereinafter "crystalline polyester resins" and "crystalline resins" encompass both crystalline resins and semicrystalline resins, unless otherwise specified.

15 In embodiments, the crystalline polyester resin is a saturated crystalline polyester resin or an unsaturated crystalline polyester resin.

The crystalline polyester resins, which are available from a number of sources, may possess various melting points of, for 20 example, from about 30° C. to about 120° C., in embodiments from about 50° C. to about 90° C. The crystalline resins may have, for example, a number average molecular weight ( $M_n$ ), as measured by gel permeation chromatography (GPC) of, for example, from about 1,000 to about 50,000, in embodiments from about 2,000 to about 25,000, in embodiments from about 3,000 to about 6,000 to about 12,000. The weight average molecular weight ( $M_w$ ) of the resin is 50,000 or less, for example, from about 2,000 to about 50,000, in embodiments from about 3,000 to about 30,000, in embodiments from about 10,000 to about 30,000 and in embodiments from about 21,000 to about 24,000, as determined by GPC using polystyrene standards. The molecular weight distribution ( $M_w/M_n$ ) of the crystalline resin is, for example, from about 2 to about 6, in embodiments from about 3 to about 4. The crystalline polyester resins may have an acid value of about 2 to about 20 mg KOH/g, in embodiments from about 5 to about 15 mg KOH/g, and in embodiments from about 8 to about 13 mg KOH/g. The acid value (or neutralization number) is the mass of potassium hydroxide (KOH) in milligrams that is required to neutralize one gram of the crystalline polyester resin.

Illustrative examples of crystalline polyester resins may include any of the various crystalline polyesters, such as poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), poly(nonylene-sebacate), poly(decylene-sebacate), poly(undecylene-sebacate), poly(dodecylene-sebacate), poly(ethylene-dodecanedioate), poly(propylene-dodecanedioate), poly(butylene-dodecanedioate), poly(pentylene-dodecanedioate), poly(hexylene-dodecanedioate), poly(octylene-dodecanedioate), poly(nonylene-dodecanedioate), poly(decylene-dodecadioate), poly(dodecylene-dodecadioate), poly(ethylene-fumarate), poly(propylene-fumarate), poly(butylene-fumarate), poly(pentylene-fumarate), poly(hexylene-fumarate), poly(octylene-fumarate), poly(nonylene-fumarate), poly(decylene-fumarate), copoly(5-sulfoisophthaloyl)-copoly(ethylene-adipate), copoly(5-sulfoisophthaloyl)-copoly(propylene-adipate), copoly(5-sulfoisophthaloyl)-copoly(butylene-adipate), copoly(5-sulfo-isophthaloyl)-copoly(pentylene-adipate), copoly(5-sulfo-isophthaloyl)-copoly(hexylene-

The crystalline resin may be prepared by a polycondensation process by reacting suitable organic diol(s) and suitable organic diacid(s) in the presence of a polycondensation catalyst. Generally, a stoichiometric equimolar ratio of organic diol and organic diacid is utilized, however, in some instances, wherein the boiling point of the organic diol is from about 180° C. to about 230° C., an excess amount of diol can be utilized and removed during the polycondensation process. The amount of catalyst utilized varies, and may be selected in an amount, for example, of from about 0.01 to about 1 mole percent of the resin. Additionally, in place of the organic diacid, an organic diester can also be selected, and where an alcohol byproduct is generated. In further embodiments, the crystalline polyester resin is a poly(dodecanoicacid-co-nonanediol).

Examples of organic diols selected for the preparation of crystalline polyester resins include aliphatic diols with from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,12-dodecanediol, and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like. The aliphatic diol is, for example, selected in an amount of from about 45 to about 50 mole percent of the resin, and the alkali sulfo-aliphatic diol can be selected in an amount of from about 1 to about 10 mole percent of the resin.

Examples of organic diacids or diesters selected for the preparation of the crystalline polyester resins include oxalic acid, succinic acid, glutaric acid, adipic acid, suberic acid, azelaic acid, sebamic acid, phthalic acid, isophthalic acid, terephthalic acid, naphthalene-2,6-dicarboxylic acid, naphthalene-2,7-dicarboxylic acid, cyclohexane dicarboxylic acid, malonic acid and mesaconic acid, a diester or anhydride thereof; and an alkali sulfo-organic diacid such as the sodio, lithio or potassium salt of dimethyl-5-sulfo-isophthalate, dialkyl-5-sulfo-isophthalate-4-sulfo-1,8-naphthalic anhydride, 4-sulfo-phthalic acid, dimethyl-4-sulfo-phthalate, dialkyl-4-sulfo-phthalate, 4-sulfophenyl-3,5-dicar-

10 Suitable crystalline polyester resins include those disclosed in U.S. Pat. No. 7,329,476 and U.S. Patent Application Pub. Nos. 2006/0216626, 2008/0107990, 2008/0236446 and 2009/0047593, each of which is hereby incorporated by reference in their entirety. In embodiments, a suitable crystalline 15 resin may include a resin composed of ethylene glycol or nonanediol and a mixture of dodecanedioic acid and fumaric acid co-monomers with the following formula (II):



23 wherein b is from about 5 to about 2000 and d is from about 5 to about 2000.

If semicrystalline polyester resins are employed herein, the semicrystalline resin may include poly(3-methyl-1-butene), poly(hexamethylene carbonate), poly(ethylene-p-carboxy phenoxy-butylate), poly(ethylene-vinyl acetate), poly(docosyl acrylate), poly(dodecyl acrylate), poly(octadecyl acrylate), poly(octadecyl methacrylate), poly(behenylpolyethoxyethyl methacrylate), poly(ethylene adipate), poly(decamethylene adipate), poly(decamethylene azelaate), poly(hexamethylene oxalate), poly(decamethylene oxalate), poly(ethylene oxide), poly(propylene oxide), poly(butadiene oxide), poly(decamethylene oxide), poly(decamethylene sulfide), poly(decamethylene disulfide), poly(ethylene sebacate), poly(decamethylene sebacate), poly(ethylene suberate), poly(decamethylene succinate), poly(eicosamethylene malonate), poly(ethylene-p-carboxy phenoxy-undecanoate), poly(ethylene dithionesophthalate), poly(methyl ethylene terephthalate), poly(ethylene-p-carboxy phenoxy-valerate), poly(hexamethylene-4,4'-oxydibenzoate), poly(10-hydroxy capric acid), poly(isophthalaldehyde), poly(octamethylene dodecanedioate), poly(dimethyl siloxane), poly(dipropyl siloxane), poly(tetramethylene phenylene diacetate), poly(tetramethylene trithiocarboxylate), poly(trimethylene dodecane dioate), poly(m-xylene), poly(p-xylylene pimelamide), and combinations thereof.

The amount of the crystalline polyester resin in a toner particle of the present disclosure, whether in core, shell or both, may be present in an amount of from 1 to about 15 percent by weight, in embodiments from about 5 to about 10 percent by weight, and in embodiments from about 6 to about 8 percent by weight, of the toner particles (that is, toner particles exclusive of external additives and water).

In embodiments, a toner of the present disclosure may also include at least one high molecular weight branched or cross-linked amorphous polyester resin. This high molecular weight resin may include, in embodiments, for example, a branched amorphous resin or amorphous polyester, a cross-linked amorphous resin or amorphous polyester, or mixtures thereof, or a non-cross-linked amorphous polyester resin that has been subjected to cross-linking. In accordance with the present disclosure, from about 1% by weight to about 100%

by weight of the high molecular weight amorphous polyester resin may be branched or cross-linked, in embodiments from about 2% by weight to about 50% by weight of the higher molecular weight amorphous polyester resin may be branched or cross-linked.

As used herein, the high molecular weight amorphous polyester resin may have, for example, a number average molecular weight ( $M_n$ ), as measured by gel permeation chromatography (GPC) of, for example, from about 1,000 to about 10,000, in embodiments from about 2,000 to about 9,000, in embodiments from about 3,000 to about 8,000, and in embodiments from about 6,000 to about 7,000. The weight average molecular weight ( $M_w$ ) of the resin is greater than 55,000, for example, from about 55,000 to about 150,000, in embodiments from about 60,000 to about 100,000, in embodiments from about 63,000 to about 94,000, and in embodiments from about 68,000 to about 85,000, as determined by GPC using polystyrene standard. The polydispersity index (PD) is above about 4, such as, for example, greater than about 4, in embodiments from about 4 to about 20, in embodiments from about 5 to about 10, and in embodiments from about 6 to about 8, as measured by GPC versus standard polystyrene reference resins. (The PD index is the ratio of the weight-average molecular weight ( $M_w$ ) and the number-average molecular weight ( $M_n$ ).) The low molecular weight amorphous polyester resins may have an acid value of from about 8 to about 20 mg KOH/g, in embodiments from about 9 to about 16 mg KOH/g, and in embodiments from about 11 to about 15 mg KOH/g. The high molecular weight amorphous polyester resins, which are available from a number of sources, can possess various melting points of, for example, from about 30° C. to about 140° C., in embodiments from about 75° C. to about 130° C., in embodiments from about 100° C. to about 125° C., and in embodiments from about 115° C. to about 121° C.

The high molecular weight amorphous resins, which are available from a number of sources, can possess various onset glass transition temperatures ( $T_g$ ) of, for example, from about 40° C. to about 80° C., in embodiments from about 50° C. to about 70° C., and in embodiments from about 54° C. to about 68° C., as measured by differential scanning calorimetry (DSC). The linear and branched amorphous polyester resins, in embodiments, may be a saturated or unsaturated resin.

The high molecular weight amorphous polyester resins may be prepared by branching or cross-linking linear polyester resins. Branching agents can be utilized, such as trifunctional or multifunctional monomers, which agents usually increase the molecular weight and polydispersity of the polyester. Suitable branching agents include glycerol, trimethylol ethane, trimethylol propane, pentaerythritol, sorbitol, diglycerol, trimellitic acid, trimellitic anhydride, pyromellitic acid, pyromellitic anhydride, 1,2,4-cyclohexanetricarboxylic acid, 2,5,7-naphthalenetricarboxylic acid, 1,2,4-butanetricarboxylic acid, combinations thereof, and the like. These branching agents can be utilized in effective amounts of from about 0.1 mole percent to about 20 mole percent based on the starting diacid or diester used to make the resin.

Compositions containing modified polyester resins with a polybasic carboxylic acid which may be utilized in forming high molecular weight polyester resins include those disclosed in U.S. Pat. No. 3,681,106, as well as branched or cross-linked polyesters derived from polyvalent acids or alcohols as illustrated in U.S. Pat. Nos. 4,863,825; 4,863,824; 4,845,006; 5,143,809; 5,057,596; 4,988,794; 4,981,939; 4,980,448; 4,933,252; 4,931,370; 4,917,983 and 4,973,539, the disclosures of each of which are incorporated by reference herein in their entirety.

In embodiments, cross-linked polyesters resins may be made from linear amorphous polyester resins that contain sites of unsaturation that can react under free-radical conditions. Examples of such resins include those disclosed in U.S.

5 Pat. Nos. 5,227,460; 5,376,494; 5,480,756; 5,500,324; 5,601, 960; 5,629,121; 5,650,484; 5,750,909; 6,326,119; 6,358,657; 6,359,105; and 6,593,053, the disclosures of each of which are incorporated by reference in their entirety. In embodiments, suitable unsaturated polyester base resins may be prepared from diacids and/or anhydrides such as, for example, maleic anhydride, terephthalic acid, trimellitic acid, fumaric acid, and the like, and combinations thereof, and diols such as, for example, bisphenol-A ethyleneoxide adducts, bisphenol A-propylene oxide adducts, and the like, and combinations thereof. In embodiments, a suitable polyester is poly (propoxylated bisphenol A co-fumaric acid).

In embodiments, a cross-linked branched polyester may be utilized as a high molecular weight amorphous polyester resin. Such polyester resins may be formed from at least two pre-gel compositions including at least one polyol having two or more hydroxyl groups or esters thereof, at least one aliphatic or aromatic polyfunctional acid or ester thereof, or a mixture thereof having at least three functional groups; and 10 optionally at least one long chain aliphatic carboxylic acid or ester thereof, or aromatic monocarboxylic acid or ester thereof, or mixtures thereof. The two components may be reacted to substantial completion in separate reactors to produce, in a first reactor, a first composition including a pre-gel having carboxyl end groups, and in a second reactor, a second composition including a pre-gel having hydroxyl end groups. The two compositions may then be mixed to create a cross-linked branched polyester high molecular weight resin. Examples of such polyesters and methods for their synthesis 15 include those disclosed in U.S. Pat. No. 6,592,913, the disclosure of which is hereby incorporated by reference in its entirety.

In embodiments, the cross-linked branched polyesters for the high molecular weight amorphous polyester resin may include those resulting from the reaction of dimethylterephthalate, 1,3-butanediol, 1,2-propanediol, and pentaerythritol.

Suitable polyols may contain from about 2 to about 100 carbon atoms and have at least two or more hydroxy groups, or esters thereof. Polyols may include glycerol, pentaerythritol, polyglycol, polyglycerol, and the like, or mixtures thereof. The polyol may include a glycerol. Suitable esters of glycerol include glycerol palmitate, glycerol sebacate, glycerol adipate, triacetin tripropionin, and the like. The polyol may be present in an amount of from about 20% to about 30% weight of the reaction mixture, in embodiments, from about 22% to about 26% weight of the reaction mixture.

Aliphatic polyfunctional acids having at least two functional groups may include saturated and unsaturated acids containing from about 2 to about 100 carbon atoms, or esters thereof, in some embodiments, from about 4 to about 20 carbon atoms. Other aliphatic polyfunctional acids include malonic, succinic, tartaric, malic, citric, fumaric, glutaric, adipic, pimelic, sebacic, suberic, azelaic, sebacic, and the like, or mixtures thereof. Other aliphatic polyfunctional acids 55 which may be utilized include dicarboxylic acids containing a  $C_3$  to  $C_6$  cyclic structure and positional isomers thereof, and include cyclohexane dicarboxylic acid, cyclobutane dicarboxylic acid or cyclopropane dicarboxylic acid.

Aromatic polyfunctional acids having at least two functional groups which may be utilized include terephthalic, isophthalic, trimellitic, pyromellitic and naphthalene 1,4-, 60 2,3-, and 2,6-dicarboxylic acids.

## 11

The aliphatic polyfunctional acid or aromatic polyfunctional acid may be present in an amount of from about 40% to about 65% weight of the reaction mixture, in embodiments, from about 44% to about 60% weight of the reaction mixture.

Long chain aliphatic carboxylic acids or aromatic monocarboxylic acids may include those containing from about 12 to about 26 carbon atoms, or esters thereof, in embodiments, from about 14 to about 18 carbon atoms. Long chain aliphatic carboxylic acids may be saturated or unsaturated. Suitable saturated long chain aliphatic carboxylic acids may include lauric, myristic, palmitic, stearic, arachidic, cerotic, and the like, or combinations thereof. Suitable unsaturated long chain aliphatic carboxylic acids may include dodecrylic, palmitoleic, oleic, linoleic, linolenic, erucic, and the like, or combinations thereof. Aromatic monocarboxylic acids may include benzoic, naphthoic, and substituted naphthoic acids. Suitable substituted naphthoic acids may include naphthoic acids substituted with linear or branched alkyl groups containing from about 1 to about 6 carbon atoms such as 1-methyl-2-naphthoic acid and/or 2-isopropyl-1-naphthoic acid. The long chain aliphatic carboxylic acid or aromatic monocarboxylic acids may be present in an amount of from about 0% to about 70% weight of the reaction mixture, in embodiments, from about 15% to about 30% weight of the reaction mixture.

Additional polyols, ionic species, oligomers, or derivatives thereof, may be used if desired. These additional glycols or polyols may be present in amounts of from about 0% to about 50% weight percent of the reaction mixture. Additional polyols or their derivatives thereof may include propylene glycol, 1,3-butanediol, 1,3-propanediol, 1,4-butanediol, 1,6-hexanediol diethylene glycol, 1,4-cyclohexanediol, 1,4-cyclohexanediethanol, neopentyl glycol, triacetin, trimethylolpropane, pentaerythritol, cellulose ethers, cellulose esters, such as cellulose acetate, sucrose acetate iso-butyrate and the like.

In embodiments, the high molecular weight resin, for example a branched polyester, may be present on the surface of toner particles of the present disclosure. The high molecular weight resin on the surface of the toner particles may also be particulate in nature, with high molecular weight resin particles having a diameter of from about 100 nanometers to about 300 nanometers, in embodiments from about 110 nanometers to about 150 nanometers.

The amount of high molecular weight amorphous polyester resin in a toner particle of the present disclosure, whether in the core, any shell, or both, may be from about 25% to about 50% by weight of the toner, in embodiments from about 30% to about 45% by weight, in other embodiments or from about 40% to about 43% by weight of the toner (that is, toner particles exclusive of external additives and water).

The ratio of crystalline resin to the low molecular weight amorphous resin to high molecular weight amorphous polyester resin can be in the range from about 1:1:98 to about 98:1:1 to about 1:98:1, in embodiments from about 1:5:5 to about 1:9:9, in embodiments from about 1:6:6 to about 1:8:8. Surfactants

In embodiments, resins, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants may be selected from ionic surfactants and nonionic surfactants. Anionic surfactants and cationic surfactants are

## 12

encompassed by the term "ionic surfactants." In embodiments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy)ethanol, available from Rhone-Poulenc as IGEPAL CA-210<sup>TM</sup>, IGEPAL CA520<sup>TM</sup>, IGEPAL CA720<sup>TM</sup>, IGEPAL CO890<sup>TM</sup>, IGEPAL CO720<sup>TM</sup>, IGEPAL CO-290<sup>TM</sup>, IGEPAL CA210<sup>TM</sup>, ANTAROX 890<sup>TM</sup> and ANTAROX 897<sup>TM</sup>. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecylbenzene sulfonate, dialkyl benzenealkyl sulfates and sulfonates, acids such as abitic acid available from Aldrich, NEOGEN R<sup>TM</sup>, NEOGEN S<sup>TM</sup> obtained from Daiichi Kogyo Seiyaku, combinations thereof, and the like. Other suitable anionic surfactants include, in embodiments, DOWFAX<sup>TM</sup> 2A1, an alkylidiphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecylbenzyl triethyl ammonium chloride, MIRAPOL<sup>TM</sup> and ALKAQUAT<sup>TM</sup>, available from Alkaril Chemical Company, SANIZOL<sup>TM</sup> (benzalkonium chloride), available from Kao Chemicals, and the like, and mixtures thereof.

## Toner

The resin of the resin emulsions described above, in embodiments a polyester resin, may be utilized to form toner compositions. Such toner compositions may include optional colorants, optional waxes, and other additives. Toners may be formed utilizing any method within the purview of those skilled in the art including, but not limited to, emulsion aggregation methods.

## Colorants

The latex particles produced as described above may be added to a colorant to produce a toner. In embodiments the colorant may be in a dispersion. The colorant dispersion may include, for example, submicron colorant particles having a size of, for example, from about 50 to about 500 nanometers in volume average diameter and, in embodiments, of from about 100 to about 400 nanometers in volume average diameter. The colorant particles may be suspended in an aqueous water phase containing an anionic surfactant, a nonionic sur-

factant, or combinations thereof. Suitable surfactants include any of those surfactants described above. In embodiments, the surfactant may be ionic and may be present in a dispersion in an amount from about 0.1 to about 25 percent by weight of the colorant, and in embodiments from about 1 to about 15 percent by weight of the colorant.

Colorants useful in forming toners in accordance with the present disclosure include pigments, dyes, mixtures of pigments and dyes, mixtures of pigments, mixtures of dyes, and the like. The colorant may be, for example, carbon black, cyan, yellow, magenta, red, orange, brown, green, blue, violet, or mixtures thereof.

In embodiments wherein the colorant is a pigment, the pigment may be, for example, carbon black, phthalocyanines, quinacridones or RHODAMINE B™ type, red, green, orange, brown, violet, yellow, fluorescent colorants, and the like.

Exemplary colorants include carbon black like REGAL 330® magnetites; Mobay magnetites including MO8029™, MO8060™; Columbian magnetites; MAPICO BLACK™ and surface treated magnetites; Pfizer magnetites including CB4799™, CB5300™, CB5600™, MCX6369™; Bayer magnetites including, BAYFERROX 8600™, 8610™; Northern Pigments magnetites including, NP604™, NP608™; Magnox magnetites including TMB-100™, or TMB-104™, HELIOGEN BLUE L6900™, D6840™, D7080™, D7020™, PYLAM OIL BLUE™, PYLAM OIL YELLOW™, PIGMENT BLUE 1™ available from Paul Uhlrich and Company, Inc.; PIGMENT VIOLET 1™, PIGMENT RED 48™, LEMON CHROME YELLOW DCC 1026™, E.D. TOLUIDINE RED™ and BON RED C™ available from Dominion Color Corporation, Ltd., Toronto, Ontario; NOVAPERM YELLOW FGL™, HOSTAPERM PINK E™ from Hoechst; and CINQUASIA MAGENTA™ available from E.I. DuPont de Nemours and Company. Other colorants include 2,9-dimethyl-substituted quinacridone and anthraquinone dye identified in the Color Index as CI 60710, CI Dispersed Red 15, diazo dye identified in the Color Index as CI 26050, CI Solvent Red 19, copper tetra(octadecyl sulfonamido) phthalocyanine, x-copper phthalocyanine pigment listed in the Color Index as CI 74160, CI Pigment Blue, Anthrathrene Blue identified in the Color Index as CI 69810, Special Blue X-2137, diarylide yellow 3,3-dichlorobenzidine acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33, 2,5-dimethoxy-4-sulfonanilide phenylazo-4'-chloro-2,5-dimethoxy acetoacetanilide, Yellow 180 and Permanent Yellow FGL. Organic soluble dyes having a high purity for the purpose of color gamut which may be utilized include Neopen Yellow 075, Neopen Yellow 159, Neopen Orange 252, Neopen Red 336, Neopen Red 335, Neopen Red 366, Neopen Blue 808, Neopen Black X53, Neopen Black X55, wherein the dyes are selected in various suitable amounts, for example from about 0.5 to about 20 percent by weight of the toner, in embodiments, from about 5 to about 18 weight percent of the toner.

In embodiments, colorant examples include Pigment Blue 15:3 having a Color Index Constitution Number of 74160, Magenta Pigment Red 81:3 having a Color Index Constitution Number of 45160:3, Yellow 17 having a Color Index Constitution Number of 21105, and known dyes such as food dyes, yellow, blue, green, red, magenta dyes, and the like.

In other embodiments, a magenta pigment, Pigment Red 122 (2,9-dimethylquinacridone), Pigment Red 185, Pigment Red 192, Pigment Red 202, Pigment Red 206, Pigment Red

235, Pigment Red 269, combinations thereof, and the like, may be utilized as the colorant.

In embodiments, toners of the present disclosure may have high pigment loadings. As used herein, high pigment loadings include, for example, toners having a colorant in an amount of from about 4 percent by weight of the toner to about 40 percent by weight of the toner, in embodiments from about 5 percent by weight of the toner to about 15 percent by weight of the toner. These high pigment loadings may be important for certain colors such as Magenta, Cyan, Black, PANTONE® Orange, Process Blue, PANTONE® yellow, and the like. (The PANTONE® colors refer to one of the most popular color guides illustrating different colors, wherein each color is associated with a specific formulation of colorants, and is published by PANTONE, Inc., of Moonachie, N.J.) One issue with high pigment loading is that it may reduce the ability of the toner particles to spherodize, that is, become circular, during the coalescence step, even at a very low pH.

The resulting latex, optionally in a dispersion, and colorant dispersion may be stirred and heated to a temperature of from about 35° C. to about 70° C., in embodiments of from about 40° C. to about 65° C., resulting in toner aggregates of from about 2 microns to about 10 microns in volume average diameter, and in embodiments of from about 5 microns to about 8 microns in volume average diameter.

#### Wax

Optionally, a wax may also be combined with the resin in forming toner particles. When included, the wax may be present in an amount of, for example, from about 1 weight percent to about 25 weight percent of the toner particles, in embodiments from about 5 weight percent to about 20 weight percent of the toner particles.

Waxes that may be selected include waxes having, for example, a weight average molecular weight of from about 500 to about 20,000, in embodiments from about 1,000 to about 10,000. Waxes that may be used include, for example, polyolefins such as polyethylene, polypropylene, and polybutene waxes such as commercially available from Allied Chemical and Petrolite Corporation, for example POLY-WAX™ polyethylene waxes from Baker Petrolite, wax emulsions available from Michaelman, Inc. and the Daniels Products Company, EPOLENE N-15™ commercially available from Eastman Chemical Products, Inc., and VISCOL 550-P™, a low weight average molecular weight polypropylene available from Sanyo Kasei K. K.; plant-based waxes, such as carnauba wax, rice wax, candelilla wax, sumacs wax, and jojoba oil; animal-based waxes, such as beeswax; mineral-based waxes and petroleum-based waxes, such as montan wax, ozokerite, ceresin, paraffin wax, microcrystalline wax, and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride distearate, and pentaerythritol tetra behenate; ester waxes obtained from higher fatty acid and multivalent alcohol multimers, such as diethyleneglycol monostearate, dipropylene-glycol distearate, diglyceryl distearate, and triglyceryl tetra-stearate; sorbitan higher fatty acid ester waxes, such as sorbitan monostearate, and cholesterol higher fatty acid ester waxes, such as cholestryl stearate. Examples of functionalized waxes that may be used include, for example, amines, amides, for example AQUA SUPERSLIP 6550™, SUPERSLIP 6530™ available from Micro Powder Inc., fluorinated waxes, for example POLYFLUO 190™, POLYFLUO 200™, POLYSILK 19™, POLYSILK 14™ available from Micro Powder Inc., mixed fluorinated, amide waxes, for example

MICROSPERSION 19<sup>TM</sup> also available from Micro Powder Inc., imides, esters, quaternary amines, carboxylic acids or acrylic polymer emulsion, for example JONCRYL 74<sup>TM</sup>, 89<sup>TM</sup>, 130<sup>TM</sup>, 537<sup>TM</sup>, and 538<sup>TM</sup>, all available from SC Johnson Wax, and chlorinated polypropylenes and polyethylenes available from Allied Chemical and Petrolite Corporation and SC Johnson wax. Mixtures and combinations of the foregoing waxes may also be used in embodiments. Waxes may be included as, for example, fuser roll release agents.

#### Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Pat. Nos. 5,290,654 and 5,302,486, the disclosures of each of which are hereby incorporated by reference in their entirety. In embodiments, toner compositions and toner particles may be prepared by aggregation and coalescence processes in which small-size resin particles are aggregated to the appropriate toner particle size and then coalesced to achieve the final toner-particle shape and morphology.

In embodiments, toner compositions may be prepared by emulsion-aggregation processes, such as a process that includes aggregating a mixture of an optional wax and any other desired or required additives, and emulsions including the resins described above, optionally in surfactants as described above, and then coalescing the aggregate mixture. A mixture may be prepared by adding an optional wax or other materials, which may also be optionally in a dispersion (s) including a surfactant, to the emulsion, which may be a mixture of two or more emulsions containing the resin. The pH of the resulting mixture may be adjusted by an acid such as, for example, acetic acid, nitric acid or the like. In embodiments, the pH of the mixture may be adjusted to from about 2 to about 4.5. Additionally, in embodiments, the mixture may be homogenized. If the mixture is homogenized, homogenization may be accomplished by mixing at about 600 to about 4,000 revolutions per minute. Homogenization may be accomplished by any suitable means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a divalent cation or a multivalent cation material. The aggregating agent may be, for example, polyaluminum halides such as polyaluminum chloride (PAC), or the corresponding bromide, fluoride, or iodide, polyaluminum silicates such as polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (Tg) of the resin.

The aggregating agent may be added to the mixture utilized to form a toner in an amount of, for example, from about 0.1% to about 8% by weight, in embodiments from about 0.2% to about 5% by weight, in other embodiments from about 0.5%

to about 5% by weight, of the resin in the mixture. This provides a sufficient amount of agent for aggregation.

In order to control aggregation and coalescence of the particles, in embodiments the aggregating agent may be metered into the mixture over time. For example, the agent may be metered into the mixture over a period of from about 5 to about 240 minutes, in embodiments from about 30 to about 200 minutes. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from about 35° C. to about 70° C.

The particles may be permitted to aggregate until a predetermined desired particle size is obtained. A predetermined desired size refers to the desired particle size to be obtained as determined prior to formation, and the particle size being monitored during the growth process until such particle size is reached. Samples may be taken during the growth process and analyzed, for example with a Coulter Counter, for average particle size. The aggregation thus may proceed by maintaining the elevated temperature, or slowly raising the temperature to, for example, from about 40° C. to about 100° C., and holding the mixture at this temperature for a time from about 0.5 hours to about 6 hours, in embodiments from about hour 1 to about 5 hours, while maintaining stirring, to provide the aggregated particles. Once the predetermined desired particle size is reached, then the growth process is halted. In embodiments, the predetermined desired particle size is within the toner particle size ranges mentioned above.

The growth and shaping of the particles following addition of the aggregation agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for example of from about 40° C. to about 90° C., in embodiments from about 45° C. to about 80° C., which may be below the glass transition temperature of the resin as discussed above.

#### Shell Resin

In embodiments, after aggregation, but prior to coalescence, a shell may be applied to the aggregated particles.

Resins which may be utilized to form the shell include, but are not limited to, the amorphous resins described above for use in the core. Such an amorphous resin may be a low molecular weight resin, a high molecular weight resin, or combinations thereof. In embodiments, an amorphous resin which may be used to form a shell in accordance with the present disclosure may include an amorphous polyester of formula I above.

In some embodiments, the amorphous resin utilized to form the shell may be crosslinked. For example, crosslinking may be achieved by combining an amorphous resin with a crosslinker, sometimes referred to herein, in embodiments, as an initiator. Examples of suitable crosslinkers include, but are not limited to, for example free radical or thermal initiators such as organic peroxides and azo compounds described above as suitable for forming a gel in the core. Examples of suitable organic peroxides include diacyl peroxides such as, for example, decanoyl peroxide, lauroyl peroxide and benzoyl peroxide, ketone peroxides such as, for example, cyclohexanone peroxide and methyl ethyl ketone, alkyl peroxyesters such as, for example, t-butyl peroxy neodecanoate, 2,5-

dimethyl 2,5-di(2-ethyl hexanoyl peroxy)hexane, t-amyl peroxy 2-ethyl hexanoate, t-butyl peroxy 2-ethyl hexanoate, t-butyl peroxy acetate, t-amyl peroxy acetate, t-butyl peroxy benzoate, t-amyl peroxy benzoate, oo-t-butyl o-isopropyl mono peroxy carbonate, 2,5-dimethyl 2,5-di(benzoyl peroxy)hexane, oo-t-butyl o-(2-ethyl hexyl)mono peroxy carbonate, and oo-t-amyl o-(2-ethyl hexyl)mono peroxy carbonate, alkyl peroxides such as, for example, dicumyl peroxide, 2,5-dimethyl 2,5-di(t-butyl peroxy)hexane, t-butyl cumyl peroxide,  $\alpha$ - $\alpha$ -bis(t-butyl peroxy)diisopropyl benzene, di-t-butyl peroxide and 2,5-dimethyl 2,5-di(t-butyl peroxy)hexyne-3, alkyl hydroperoxides such as, for example, 2,5-dihydro peroxy 2,5-dimethyl hexane, cumene hydroperoxide, t-butyl hydroperoxide and t-amyl hydroperoxide, and alkyl peroxyketals such as, for example, n-butyl 4,4-di(t-butyl peroxy)valerate, 1,1-di(t-butyl peroxy)3,3,5-trimethyl cyclohexane, 1,1-di(t-butyl peroxy)cyclohexane, 1,1-di(t-amyl peroxy)cyclohexane, 2,2-di(t-butyl peroxy)butane, ethyl 3,3-di(t-butyl peroxy)butyrate and ethyl 3,3-di(t-amyl peroxy)butyrate, and combinations thereof. Examples of suitable azo compounds include 2,2'-azobis(2,4-dimethylpentane nitrile), azobis-isobutyronitrile, 2,2'-azobis(isobutyronitrile), 2,2'-azobis(2,4-dimethyl valeronitrile), 2,2'-azobis(methyl butyronitrile), 1,1'-azobis(cyano cyclohexane), other similar known compounds, and combinations thereof.

The crosslinker and amorphous resin may be combined for a sufficient time and at a sufficient temperature to form the crosslinked polyester gel. In embodiments, the crosslinker and amorphous resin may be heated to a temperature of from about 25° C. to about 99° C., in embodiments from about 30° C. to about 95° C., for a period of time of from about 1 minute to about 10 hours, in embodiments from about 5 minutes to about 5 hours, to form a crosslinked polyester resin or polyester gel suitable for use as a shell.

Where utilized, the crosslinker may be present in an amount of from about 0.001% by weight to about 5% by weight of the resin, in embodiments from about 0.01% by weight to about 1% by weight of the resin. The amount of CCA may be reduced in the presence of crosslinker or initiator.

A single polyester resin may be utilized as the shell or, as noted above, in embodiments a first polyester resin may be combined with other resins to form a shell. Multiple resins may be utilized in any suitable amounts. In embodiments, a first amorphous polyester resin, for example a low molecular weight amorphous resin of formula I above, may be present in an amount of from about 20 percent by weight to about 100 percent by weight of the total shell resin, in embodiments from about 30 percent by weight to about 90 percent by weight of the total shell resin. Thus, in embodiments a second resin, in embodiments a high molecular weight amorphous resin, may be present in the shell resin in an amount of from about 0 percent by weight to about 80 percent by weight of the total shell resin, in embodiments from about 10 percent by weight to about 70 percent by weight of the shell resin.

#### Coalescence

The mixture of latex, colorant, optional wax, and any additives, is subsequently coalesced. Coalescing may include stirring and heating at a temperature of from about 80° C. to about 99° C., for a period of from about 0.5 to about 12 hours, and in embodiments from about 1 to about 6 hours. Coalescing may be accelerated by additional stirring.

As noted above, one issue with high pigment loading for toners of the present disclosure is that it may reduce the ability of the toner to spherodize during the coalescence step, even at a very low pH. Thus, in embodiments, a metal compound may be added during the coalescence process. The metal may be in

the form of a metal compound such as a metal salt, oxide, and/or hydroxide. In embodiments, a metal compound, such as a transition metal powder and/or a transition metal salt, may be added to the mixture of latex, colorant, optional wax, and any additives, at the beginning of the coalescence process. Suitable metals include, for example, copper, zinc, iron, cobalt, nickel, molybdenum, manganese, chromium, vanadium, and/or titanium, as well as metal alloys such as copper/zinc alloys.

In other embodiments, elemental copper or copper compounds, including salts, iron or iron compounds, including salts, or combinations thereof, may be utilized to speed coalescence and obtain desired particle circularity for a toner of the present disclosure. Examples of such copper and/or iron compounds, including salts, include nitrates, sulfates, halides, acetates, phosphates, oxides, hydroxides, carbonates, combinations thereof, and the like. In embodiments, the compound, such as a salt, may be insoluble. The degree of solubility may be, for example:

20 nitrates—soluble  
sulfates—soluble  
halides—soluble  
acetates—soluble  
phosphates—insoluble  
25 oxides—insoluble  
hydroxides—insoluble  
carbonates—insoluble

In embodiments, a copper nitrate, such as copper II nitrate, may be utilized as the metal salt. In other embodiments, an iron salt such as iron nitrate may be utilized as the metal salt.

30 The amount of metal powder added to the mixture may be from about 0.01 weight percent to about 4 weight percent, in embodiments from about 0.09 to about 1 weight percent. The amount of metal salt added to the mixture may be from about 0.01 weight percent to about 4 weight percent, in embodiments from about 0.09 to about 1 weight percent.

35 The use of the transition metal powder and/or transition metal salt enables rapid coalescence of highly pigmented polyester toners. Coalescence may occur over a period of time of from about 0.1 hours to about 10 hours, in embodiments from about 0.5 hours to about 5 hours.

40 Surprisingly, the presence of the transition metal powder and/or transition metal salt may facilitate fast toner coalescence to achieve a circularity of greater than about 0.95. 45 Without this improved process, the toner circularity achieved in a highly pigmented EA toner may be less than about 0.94. The addition of the insoluble transition metal powder and/or the addition of the metal salt imparts no detrimental properties to the toner particles. In fact, very little of the metal remains in the final toner.

45 Moreover, a highly pigmented toner of the present disclosure may possess increased levels of pigment. For example, whereas a conventional magenta toner may contain about 4.5% PR122 and 4.5% PR269, a highly pigmented toner of 50 the present disclosure may contain about 6.525% of each pigment, for a total pigment loading of about 13.055 by weight.

#### Subsequent Treatments

55 In embodiments, after coalescence, the pH of the mixture may then be lowered to from about 3.5 to about 6 and, in embodiments, to from about 3.7 to about 5.5 with, for example, an acid, to further coalesce the toner aggregates. Suitable acids include, for example, nitric acid, sulfuric acid, hydrochloric acid, citric acid and/or acetic acid. The amount of acid added may be from about 0.1 to about 30 percent by weight of the mixture, and in embodiments from about 1 to about 20 percent by weight of the mixture.

The mixture may be cooled, washed and dried. Cooling may be at a temperature of from about 20° C. to about 40° C., in embodiments from about 22° C. to about 30° C., over a period of time of from about 1 hour to about 8 hours, in embodiments from about 1.5 hours to about 5 hours.

In embodiments, cooling a coalesced toner slurry may include quenching by adding a cooling media such as, for example, ice, dry ice and the like, to effect rapid cooling to a temperature of from about 20° C. to about 40° C., in embodiments of from about 22° C. to about 30° C. Quenching may be feasible for small quantities of toner, such as, for example, less than about 2 liters, in embodiments from about 0.1 liters to about 1.5 liters. For larger scale processes, such as for example greater than about 10 liters in size, rapid cooling of the toner mixture may not be feasible or practical, neither by the introduction of a cooling medium into the toner mixture, or by the use of jacketed reactor cooling.

The toner slurry may then be washed. The washing may be carried out at a pH of from about 7 to about 12, in embodiments at a pH of from about 9 to about 11. The washing may be at a temperature of from about 30° C. to about 70° C., in embodiments from about 40° C. to about 67° C. The washing may include filtering and reslurrying a filter cake including toner particles in deionized water. The filter cake may be washed one or more times by deionized water, or washed by a single deionized water wash at a pH of about 4 wherein the pH of the slurry is adjusted with an acid, and followed optionally by one or more deionized water washes.

Drying may be carried out at a temperature of from about 35° C. to about 75° C., and in embodiments of from about 45° C. to about 60° C. The drying may be continued until the moisture level of the particles is below a set target of about 1% by weight, in embodiments of less than about 0.7% by weight.

The toner of the present disclosure may possess particles having a volume average diameter (also referred to as "volume average particle diameter") of from about 3 microns to about 10 microns, in embodiments from about 3.2 microns to about 8.5 microns, in embodiments from about 3.3 microns to about 7 microns, in embodiments about 5.8 microns. As noted above, the resulting toner particles may have a circularity greater than about 0.95, in embodiments from about 0.95 to about 0.998, in embodiments from about 0.955 to about 0.97. When the spherical toner particles have a circularity in this range, the spherical toner particles remaining on the surface of the image holding member pass between the contacting portions of the imaging holding member and the contact charger, the amount of deformed toner is small, and therefore generation of toner filming can be prevented so that a stable image quality without defects can be obtained over a long period.

#### Additives

In embodiments, the toner particles may also contain other optional additives, as desired or required. For example, the toner may include positive or negative charge control agents, for example in an amount of from about 0.1 to about 10 percent by weight of the toner, in embodiments from about 1 to about 3 percent by weight of the toner. Examples of suitable charge control agents include quaternary ammonium compounds inclusive of alkyl pyridinium halides; bisulfates; alkyl pyridinium compounds, including those disclosed in U.S. Pat. No. 4,298,672, the disclosure of which is hereby incorporated by reference in its entirety; organic sulfate and sulfonate compositions, including those disclosed in U.S. Pat. No. 4,338,390, the disclosure of which is hereby incorporated by reference in its entirety; cetyl pyridinium tetrafluoroborates; distearyl dimethyl ammonium methyl sulfate; aluminum salts such as BONTRON E84<sup>TM</sup> or E88<sup>TM</sup> (Hodogaya

Chemical); combinations thereof, and the like. Such charge control agents may be applied simultaneously with the shell resin described above or after application of the shell resin.

There can also be blended with the toner particles external additive particles including flow aid additives, which additives may be present on the surface of the toner particles. Examples of these additives include metal oxides such as titanium oxide, silicon oxide, tin oxide, mixtures thereof, and the like; colloidal and amorphous silicas, such as AEROSIL<sup>®</sup>, metal salts and metal salts of fatty acids inclusive of zinc stearate, aluminum oxides, cerium oxides, and mixtures thereof. Each of these external additives may be present in an amount of from about 0.1 percent by weight to about 5 percent by weight of the toner, in embodiments of from about 0.25 percent by weight to about 3 percent by weight of the toner. Suitable additives include those disclosed in U.S. Pat. Nos. 3,590,000, 3,800,588, and 6,214,507, the disclosures of each of which are hereby incorporated by reference in their entirety. Again, these additives may be applied simultaneously with a shell resin described above or after application of the shell resin.

In embodiments, toners of the present disclosure may be utilized as ultra low melt (ULM) toners. In embodiments, the dry toner particles, exclusive of external surface additives, may have the following characteristics:

- (1) Number Average Geometric Standard Deviation (GSD<sub>n</sub>) and/or Volume Average Geometric Standard Deviation (GSD<sub>v</sub>) of from about 1.05 to about 1.55, in embodiments from about 1.1 to about 1.4.
- (2) Glass transition temperature of from about 40° C. to about 65° C., in embodiments from about 45° C. to about 62° C.

The characteristics of the toner particles may be determined by any suitable technique and apparatus. Volume average particle diameter D<sub>50v</sub>, GSD<sub>v</sub>, and GSD<sub>n</sub> may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3. Toners produced in accordance with the present disclosure may possess excellent relative charging characteristics when exposed to extreme relative humidity (RH) conditions. The low-humidity zone (C zone) may be about 10° C/15% RH, while the high humidity zone (A zone) may be about 28° C./85% RH. Toners of the present disclosure may also possess a parent toner charge per mass ratio (Q/m) of from about -3 µC/gram to about -90 µC/gram, in embodiments from about -10 µC/gram to about -80 µC/gram, and a final toner charging after surface additive blending of from -10 µC/gram to about -70 µC/gram, in embodiments from about -15 µC/gram to about -60 µC/gram.

#### Developers

The toner particles thus formed may be formulated into a developer composition. The toner particles may be mixed with carrier particles to achieve a two-component developer composition. The toner concentration in the developer may be from about 1% to about 25% by weight of the total weight of the developer, in embodiments from about 2% to about 15% by weight of the total weight of the developer.

#### Carriers

Examples of carrier particles that can be utilized for mixing with the toner include those particles that are capable of triboelectrically obtaining a charge of opposite polarity to that of the toner particles. Illustrative examples of suitable

carrier particles include granular zircon, granular silicon, glass, steel, nickel, ferrites, iron ferrites, silicon dioxide, and the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and the like. For example, coatings containing polyvinylidene-fluoride, available, for example, as KYNAR 301FTM, and/or polymethylmethacrylate, for example having a weight average molecular weight of about 300,000 to about 350,000, such as commercially available from Soken, may be used. In embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100  $\mu\text{m}$  in size, in embodiments from about 50 to about 75  $\mu\text{m}$  in size, coated with about 0.5% to about 10% by weight, in embodiments from about 0.7% to about 5% by weight of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

#### Imaging

The toners can be utilized for electrostatographic or electrophotographic processes, including those disclosed in U.S. Pat. No. 4,295,990, the disclosure of which is hereby incorporated by reference in its entirety. In embodiments, any

known type of image development system may be used in an image developing device, including, for example, magnetic brush development, jumping single-component development, hybrid scavengelss development (HSD), and the like. 5 These and similar development systems are within the purview of those skilled in the art.

10 Imaging processes include, for example, preparing an image with an electrophotographic device including a charging component, an imaging component, a photoconductive component, a developing component, a transfer component, and a fusing component. In embodiments, the development component may include a developer prepared by mixing a carrier with a toner composition described herein. The electrophotographic device may include a high speed printer, a black and white high speed printer, a color printer, and the like.

15 Once the image is formed with toners/developers via a suitable image development method such as any one of the aforementioned methods, the image may then be transferred 20 to an image receiving medium such as paper and the like. In embodiments, the toners may be used in developing an image in an image-developing device utilizing a fuser roll member. Fuser roll members are contact fusing devices that are within the purview of those skilled in the art, in which heat and 25 pressure from the roll may be used to fuse the toner to the image-receiving medium. In embodiments, the fuser member may be heated to a temperature above the fusing temperature of the toner, for example to temperatures of from about 70° C. to about 160° C., in embodiments from about 80° C. to about 30 150° C., in other embodiments from about 90° C. to about 140° C., after or during melting onto the image receiving substrate.

30 In embodiments where the toner resin is crosslinkable, such crosslinking may be accomplished in any suitable manner. For example, the toner resin may be crosslinked during 35 fusing of the toner to the substrate where the toner resin is crosslinkable at the fusing temperature. Crosslinking also may be effected by heating the fused image to a temperature at which the toner resin will be crosslinked, for example in a 40 post-fusing operation. In embodiments, crosslinking may be effected at temperatures of from about 160° C. or less, in embodiments from about 70° C. to about 160° C., in other embodiments from about 80° C. to about 140° C.

45 Utilizing the methods of the present disclosure, highly pigmented toners may be produced which require less toner to obtain the same image. These highly pigmented toners may exhibit an increase in pigment loading of about 45% higher than nominal. Reducing the toner mass per unit area (TMA) on the print results in a thinner toner layer. To compensate for the reduced TMA, and still get the correct optical density, the loading of pigment in the toner should be increased proportionally to the TMA reduction, so that the total amount of pigment in the image layer is the same. This reduces the toner run cost proportionally to the TMA reduction. The thinner 50 toner layers also result in more of an offset look and feel for the print, as offset inks produce thin image layers on the print.

55 Thus, as depicted in FIG. 1, as compared with a conventional toner (FIG. 1A), a toner of the present disclosure (FIG. 1B) may be highly pigmented and of a larger size, but may still provide a toner layer of desirable, lower, thickness and TMA.

Utilizing the methods of the present disclosure, as noted above, toners may be produced having a volume average diameter of from about 3 microns to about 10 microns, in 60 embodiments from about 3.3 microns to about 8.5 microns, in embodiments from about 3.3 microns to about 7 microns, in embodiments about 5.8 microns. The thickness of an image

formed with such toner, sometimes referred to herein, in embodiments, as toner pile height, or thickness for a single color 100% monolayer solid area color patch, may be from about 0.5 microns to about 7 microns, in embodiments from about 1 micron to about 6 microns, in other embodiments from about 2 microns to about 5 microns.

The following Examples are being submitted to illustrate embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 25° C.

## EXAMPLES

## Comparative Example 1

A magenta EA polyester toner was prepared with nominal amount of pigment, at a 2 liter batch size, including about 270 grams of dry toner. About 58 grams of a high molecular weight amorphous resin in an emulsion, the amorphous resin having a molecular weight of about 85,000, was combined with about 58 grams of a low molecular weight in an emulsion, the amorphous resin having a molecular weight of about 20,000. Both amorphous resins were of the following formula:



wherein m was from about 5 to about 1000.

About 18 grams of a crystalline resin in an emulsion was added thereto. The crystalline resin was of the following formula:



wherein b was from about 5 to about 2000 and d was from about 5 to about 2000. The crystalline resin was added so that it was present in an amount of about 6.7% by weight of the toner. About 12 grams of pigment in a dispersion, PR122 (about 4.5% by weight of toner) and PR269 (about 4.5% by weight of toner), and about 24 grams of a polyethylene wax (commercially available from IGI) in a dispersion (about 9% by weight of toner) were added mixed therewith and then the pH was adjusted to about 4.2 using about 0.3M nitric acid.

The slurry was then homogenized for a total of about 10 minutes at a rate of from about 3000 to about 6000 revolutions per minute (rpm) while adding about 1.35 grams of aluminum sulfate as a coagulant. The toner slurry was then transferred to the 2 liter Buchi reactor and heated to begin aggregation. The toner slurry was aggregated at a temperature of about 43° C. During aggregation, the toner particle size was closely monitored. Once the particles reached about 4.8 microns in size, a

shell including the same amorphous emulsions described above was added to achieve the final targeted particle size of about 5.8 microns. With a pH adjustment using sodium hydroxide (NaOH) and an ethylene diamine tetraacetic acid (EDTA) chelating agent (VERSENE-100), the aggregation step was frozen. The process proceeded with the reactor temperature (Tr) increased to about 85° C. while maintaining a pH  $\geq$  7.5 until the Tr was about 85° C. Once at 85° C., the pH of the toner slurry was reduced to about 7 with the addition of diluted nitric acid and held until the circularity reached  $\geq$  0.960.

Final toner particles thus produced had a particle size (D50) and circularity of 5.8 microns and 0.963, respectively.

15

## Comparative Example 2

A magenta EA polyester toner was prepared as described in Comparative Example 1 above, but this toner had about 45% higher amount of pigment. More specifically, the pigment dispersions included PR122 (about 6.525% by weight of toner) and PR269 (about 6.525% by weight of toner).

Once the Tr reached about 85° C., the pH of the toner slurry was reduced to about 7 with the addition of diluted nitric acid and held for about 3 hours. The final toner particles had a size (D50) and circularity of 5.8 microns and 0.940, respectively.

## Examples 1 and 2

(I) 30 Magenta EA polyester toners were prepared with about 45% higher amount of pigment as per Comparative Example 2, except about 0.1% copper nitrate was added at the beginning of coalescence. (Examples 1 and 2 were repeats of the same example.) More specifically, the same process was followed as per Comparative Example 2 above, except that after the aggregation step was frozen, the process proceeded with the reactor temperature (Tr) being increased while maintaining a pH  $\geq$  7.5 until Tr was about 85° C. Once at 85° C., the pH of the toner slurry was reduced to about 7 with the addition of diluted nitric acid, and copper II nitrate was added in an amount of about 0.1% by weight of the toner and held for about 3 hours (the desired circularity was obtained after about 30 minutes). The final toner particles had a particle size (D50) and circularity of 5.8 microns and 0.960, respectively.

The circularity obtained for the above toners was plotted as a function of time during coalescence as depicted in FIG. 2. As can be seen in FIG. 2, Comparative Example 1, which was the nominal pigment loading, achieved the desired circularity within 3 hours of coalescence. For Comparative Example 2, with the pigment loading increased by 45%, the toner never achieved the target circularity, even after 3 hours of coalescence. For Examples 1 and 2, which were repeats of the same process of Comparative Example 2, but with 0.1% copper nitrate added at the beginning of coalescence, the coalescence rate was dramatically increased such that the target circularity was achieved in just over 30 minutes.

## Bench Charging

Examples 1 and 2 were blended with a conventional additive package for bench charging. The additive package included the following:

The additive package utilized was as follows:

about 0.88% of titanium dioxide treated with a decylsilane, commercially available as JMT2000 from Tayca;

about 1.71% of a silica surface treated with polydimethylsiloxane, commercially available as RY50 from Evonik (from Nippon Aerosil);

## 25

about 1.73% of a sol-gel silica surface treated with hexamethylidisilazane, commercially available as X24-9163A from Nissin Chemical Kogyo;

about 0.55% of a cerium dioxide, commercially available as E10 from Mitsui Mining & Smelting; and about 0.2% of zinc stearate.

Developer samples were prepared with about 0.5 grams of the toner sample and about 10 grams of the carrier. A duplicate developer sample pair was prepared. One developer of the pair was conditioned overnight in A-zone (28° C./85% RH), and the other was conditioned overnight in the C-zone environmental chamber (10° C./15% RH). The next day, the developer samples were sealed and agitated for about 2 minutes and then about 1 hour using a Turbula mixer. After about 2 minutes and about 1 hour of mixing, the toner triboelectric charge was measured using a charge spectrograph using a 100 V/cm field. The toner charge (q/d) was measured visually as the midpoint of the toner charge distribution. The charge was reported in millimeters of displacement from the zero line. (The displacement in mm can be converted to q/d charge in femtocoulombs per micron by multiplication by 0.092 femtocoulombs/mm.) Following the 1 hour of mixing, an additional 0.5 grams of toner sample was added to the already charged developer, and mixed for a further 15 seconds, where a q/d displacement was again measured, and then mixed for a further 45 seconds (total about 1 minute of mixing), and again a q/d displacement was measured. A commercially available magenta toner from the Xerox 700 Digital Color Press, was used as a comparison. The charging results obtained for the toners of the Examples are set forth in FIG. 3, and the charging results for the commercially available magenta toner are set forth in FIG. 4. As can be seen from the Figures, the magenta toners from Examples 1 and 2 had equal or slightly better bench charging, with slightly improved relative humidity (RH) sensitivity, compared with the production magenta toner. This evidences that the copper treatment at the beginning of coalescence had no detrimental effects on the resulting toners.

## Example 3

A green polyester toner was produced with the addition of copper nitrate at the beginning of coalescence as follows. The same process was followed as per Examples 1 and 2 above, except the pigment dispersion included PG 7 (about 7.95% by weight of toner). As in Examples 1 and 2, copper II nitrate was added in an amount of about 0.1% by weight of the toner at the start of coalescence, and held for about 3 hours. The final toner particles had a particle size (D50) and circularity of 7.4 microns and 0.958, respectively.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. A process comprising:

contacting at least one polyester resin with at least one colorant, at least one surfactant, and an optional wax to form an emulsion possessing small particles;

## 26

optionally contacting the emulsion with an aggregating agent comprising a first metal compound; aggregating the small particles; halting aggregation;

adding a second metal compound comprising a metal selected from the group consisting of copper, iron, and alloys thereof to the aggregated small particles; coalescing the aggregated particles in the presence of said second metal compound to form toner particles; and recovering the toner particles, wherein the toner particles possess a volume average diameter of from about 3 microns to about 10 microns.

2. A process according to claim 1, wherein the at least one polyester resin comprises at least one amorphous polyester resin, optionally in combination with at least one crystalline polyester resin.

3. The process according to claim 2, wherein the at least one amorphous resin is of the formula:



wherein m is from about 5 to about 1000.

4. The process according to claim 2, wherein the at least one crystalline resin is of the formula:



wherein b is from about 5 to about 2000 and d is from about 5 to about 2000.

5. A process according to claim 1, wherein the second metal compound is selected from the group consisting of nitrates, sulfates, halides, acetates, phosphates, oxides, hydroxides, carbonates, and combinations thereof.

6. A process according to claim 1, wherein the second metal compound is selected from the group consisting of copper II nitrate and iron nitrate.

7. A process according to claim 1, wherein coalescing the aggregated small particles to form toner particles occurs for a period of from about 0.5 hours to about 5 hours and produces toner particles having a circularity of from about 0.95 to about 0.998.

8. A process according to claim 2, wherein the at least one amorphous resin comprises at least one low molecular weight amorphous resin in combination with at least one high molecular weight amorphous resin.

9. A process according to claim 1, wherein the at least one colorant comprises dyes, pigments, combinations of dyes, combinations of pigments, and combinations of dyes and pigments, present in an amount of from about 4 percent to about 40 percent by weight of the toner, and wherein the optional wax is selected from the group consisting of polyolefins, carnauba wax, rice wax, candelilla wax, sumacs wax, jojoba oil, beeswax, montan wax, ozokerite, ceresin, paraffin wax, microcrystalline wax, Fischer-Tropsch wax, stearyl

stearate, behenyl behenate, butyl stearate, propyl oleate, glyceride monostearate, glyceride distearate, pentaerythritol tetra behenate, diethyleneglycol monostearate, dipropyleneglycol distearate, diglyceryl distearate, triglyceryl tetra stearate, sorbitan monostearate, cholestryl stearate, and combinations thereof, present in an amount from about 0.1 percent to about 30 percent by weight of the toner.

10. A process according to claim 1, further comprising: applying the toner particles to a substrate; and fusing the toner particles to the substrate, wherein an image formed with the toner has a toner pile height from about 0.5 microns to about 7 microns.

11. A process comprising:
  - contacting at least one amorphous resin with at least one crystalline resin, at least one colorant, at least one surfactant, and an optional wax to form an emulsion possessing small particles;
  - optionally contacting the emulsion with an aggregating agent comprising a first metal compound;
  - aggregating the small particles;
  - halting aggregation;
  - adding to the aggregated small particles, a second metal compound selected from the group consisting of nitrates, sulfates, halides, acetates, phosphates, oxides, hydroxides, carbonates, and combinations thereof, possessing a metal selected from the group consisting of copper, iron, and alloys thereof;
  - coalescing the aggregated particles in the presence of said second metal compound to form toner particles; and
  - recovering the toner particles, wherein the toner particles possess a volume average diameter of from about 3 microns to about 10 microns.
12. The process according to claim 11, wherein the at least one amorphous resin is of the formula:

**12.** The process according to claim 11, wherein the at least one amorphous resin is of the formula:



wherein  $m$  is from about 5 to about 1000, and the crystalline resin is of the formula:



wherein b is from about 5 to about 2000 and d is from about 5 to about 2000.

13. A process according to claim 11, wherein the second metal compound is selected from the group consisting of copper II nitrate and iron nitrate.

14. A process according to claim 11, wherein coalescing the aggregated small particles to form toner particles occurs

for a period of from about 0.5 hours to about 5 hours and produces toner particles having a circularity of from about 0.95 to about 0.998.

15. A process according to claim 11, wherein the at least one amorphous resin comprises at least one low molecular weight amorphous resin in combination with at least one high molecular weight amorphous resin.

16. A process according to claim 11, wherein the at least one colorant comprises dyes, pigments, combinations of dyes, combinations of pigments, and combinations of dyes and pigments, present in an amount of from about 5 percent to about 15 percent by weight of the toner, and wherein the optional wax is selected from the group consisting of polyolefins, carnauba wax, rice wax, candelilla wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentaerythritol tetra behenate, diethyleneglycol monostearate, dipropyleneglycol distearate, diglyceryl distearate, triglyceryl tetrastearate, sorbitan monostearate, cholestryl stearate, and combinations thereof, present in an amount from about 0.1 percent to about 30 percent by weight of the toner.

17. A process according to claim 11, further comprising: applying the toner particles to a substrate; and fusing the toner particles to the substrate, wherein an image formed with the toner has a toner pile height from about 0.5 microns to about 7 microns.

18. A process comprising:  
contacting at least one amorphous resin with at least one crystalline resin, at least one colorant, at least one surfactant, and an optional wax to form an emulsion possessing small particles;  
contacting the emulsion with an aggregating agent comprising a first metal compound;  
aggregating the small particles;  
halting aggregation;

halting aggregation, adding to the aggregated small particles a second metal compound selected from the group consisting of nitrates, sulfates, halides, acetates, phosphates, oxides, hydroxides, carbonates, and combinations thereof, possessing a metal selected from the group consisting of copper, iron, and alloys thereof; coalescing the aggregated particles in the presence of said second metal compound for a period of time of from about 0.5 hours to about 5 hours to form toner particles; and recovering the toner particles, wherein the colorant comprises dyes, pigments, combinations of dyes, combinations of pigments, and combinations of dyes and pigments, present in an amount of from about 4 percent to about 40 percent by weight of the toner, and wherein the toner particles possess a volume average diameter of from about 3 microns to about 10 microns, and a circularity of from about 0.95 to about 0.998.

19. A process according to claim 18, wherein the second metal compound comprises copper II nitrate.

20. A process according to claim 18, further comprising: applying the toner particles to a substrate; and fusing the toner particles to the substrate, wherein an image formed with the toner has a toner pile height from about 0.5 microns to about 7 microns.

\* \* \* \*